

# United States Patent [19]

Takanishi et al.

[11] 3,859,111

[45] Jan. 7, 1975

[54] **HEAT-SENSITIVE RECORDING SHEET**

[75] Inventors: **Takashi Takanishi**, Neyagawa; **Hirosi Nishiuchi**, Kadoma, both of Japan

[73] Assignee: **General Company, Ltd.**, Osaka-shi, Osaka-fu, Japan

[22] Filed: **Dec. 3, 1973**

[21] Appl. No.: **421,142**

**Related U.S. Application Data**

[63] Continuation of Ser. No. 191,773, Oct. 22, 1971, abandoned.

**Foreign Application Priority Data**

Nov. 20, 1970 Japan ..... 45.102005

[52] U.S. Cl. .... **117/36.8**, 117/36.9

[51] Int. Cl. .... **B41m 5/18**

[58] **Field of Search** ..... 117/36.2, 36.8, 36.9

[56] **References Cited**

**UNITED STATES PATENTS**

2,663,657 12/1953 Miller et al. .... 117/36.8

|           |         |                |       |            |
|-----------|---------|----------------|-------|------------|
| 2,916,395 | 12/1959 | Owen           | ..... | 117/36.8   |
| 3,149,993 | 9/1964  | Baumann et al. | ..... | 117/36.9   |
| 3,414,423 | 12/1968 | Fierke et al.  | ..... | 117/36.8 X |
| 3,442,682 | 5/1969  | Fukawa         | ..... | 117/36.8   |

*Primary Examiner*—Thomas J. Herbert, Jr.  
*Attorney, Agent, or Firm*—Fitzpatrick, Cella, Harper & Scinto

[57]

## ABSTRACT

A heat-sensitive recording sheet having a coating layer comprising a uniform dispersion of particles of a member selected from the group consisting of the iron salts of an aliphatic acid and a member selected from the group consisting of 8-hydroxyquinoline and halogen derivatives thereof, as the color-forming reaction materials and an inhibitor of unusual color-development selected from the group consisting of ethylenediamine tetraacetic acid and alkali metal salts thereof.

**10 Claims, No Drawings**

## HEAT-SENSITIVE RECORDING SHEET

This is a continuation of application Ser. No. 191,773, filed Oct. 22, 1971, now abandoned. su

## BACKGROUND OF THE INVENTION

## 1. Field of the Invention

This invention relates to a novel heat-sensitive recording sheet. More particularly, this invention relates to a heat-sensitive recording sheet having a support with a heat-sensitive layer coated on the support. These novel heat-sensitive recording sheets can be used for reproducing originals such as books, printing matters, and drawings by a thermal reproduction system, for recording diagrams in an automatic recording device by a heat pen system, and for recording, by a thermal print head, in the recording portions of computers, calculating machines, billing machines and the like.

## 2. Description of the prior Art

Heretofore, in the prior art, various heat-sensitive sheets for reproduction systems have been known but these prior art heat-sensitive recording sheets have exhibited various disadvantages. For example, when color-forming components participating in a color-forming reaction are formed into a single coating agent, some of these agents have been found to be only slightly soluble in the solvents commonly used. A further problem sometimes occurs when finely divided metal particles become mixed with the coating agents. Since the color-forming reaction is a solid-liquid reaction or a liquid-liquid reaction, the single coating agent itself can easily color-form as a result of metal powder contamination and slight solvent solubility with the result that the contrast of the resulting image with respect to the background is so low that conventional recording paper cannot practically be used. Furthermore, the color-forming reaction often disadvantageously proceeds in the coating agent during storage and quality control of the resulting products is almost impossible. Still further, the product itself may deteriorate due to moisture present during storage and thereby become very unstable. Attempts to overcome these disadvantages by preparing the components of a two component system separately and forming two coating layers have been tried but this method still has the following drawbacks. The heat-sensitivity is usually so low that the heat-recording member cannot follow the response of the heat-sensitive recording for the short time heating (0.01 - 0.01 second) periods used in a high speed reproduction device. Also, the two layer coating is not economical from a manufacturing point of view and quality control is difficult since the product is unstable. Further, the resulting print is not clear and even if a two layer structure is employed, unusual color formation at the interface thereof cannot be inhibited.

A object of the present invention is to provide a stable heat-sensitive recording sheet free of the above-mentioned disadvantages.

Another object of this invention is to provide a method for producing a stable, heat-sensitive recording sheet by applying a single coating agent to a support to form a single layer coating heat-sensitive recording sheet.

## SUMMARY OF THE INVENTION

According to the present invention, the heat-sensitive recording sheet has a coating comprising a

uniform dispersion of particles of a component A and a component B as color-forming reaction materials and a component C which is an inhibitor of unusual color-development and is selected from the group consisting of ethylenediamine tetraacetic acid and alkali metal salts thereof. Component A is at least one member selected from the group consisting of the iron salts of aliphatic acids and component B is at least one member selected from the group consisting of 8-hydroxyquinoline and halogen derivatives thereof.

## DESCRIPTION OF THE PREFERRED EMBODIMENT

Component A is at least one member selected from the class of iron salts of aliphatic acids and is reacted with at least one or more compounds selected from the class of 8-hydroxyquinoline and halogen derivatives thereof, i.e. component B, in the presence of an inhibitor of unusual color-development to produce a black color which can then be utilized as a recording image.

Representative examples of component A are the ferrous and ferric salts of aliphatic acids. Preferred aliphatic acids include aliphatic carboxylic acids containing from about 8 to 24 carbon atoms. These include, for example, caprylic acid, pelargonic acid, capric acid, lauric acid, myristic acid, palmitic acid, stearic acid, margaric acid, arachidic acid, behenic acid, lignoceric acid, oleic acid, erucic acid, cetolic acid and the like. From a practical point of view, it is preferable to utilize aliphatic acids whose iron salts have a melting point ranging from 50°C to 170°C.

Representative examples of component B include 8-hydroxyquinoline of the formula



M.P. 75-76°C.

and halogen derivatives of 8-hydroxyquinoline such as 5, 7-dibromo-8-hydroxyquinoline of the formula



M.P. 196°C.

and 5-chloro-7-iodo-8-hydroxyquinoline of the formula



M.P. 172-178°C.

Other halogen derivatives of 8-hydroxyquinoline which may be utilized include 5-bromo-8-hydroxyquinoline, 5-iodo-8-hydroxyquinoline, 5, 7-dichloro-8-hydroxyquinoline, 5, 7-diiodo-8-hydroxyquinoline, 5-chloro-7-bromo-8-hydroxyquinoline and the like.

As component C of the present invention, i.e., the inhibitor of unusual color-development, ethylenediamine tetraacetic acid and alkali metal salts thereof, can be

utilized. Ethylenediamine tetraacetic acid is known as "EDTA" and may be represented by the formula:



Disodium or dipotassium ethylenediamine tetraacetate are the preferred alkali metal salts of "EDTA" for use in this invention.

Unusual color-forming inhibitors are used in the heat-sensitive copy-sheet of U.S. Pat. No. 3,442,682, but the specific combination of components A, B and C of the present invention is not disclosed therein. Chelating agents such as oxalic acid, citric acid, tetracetic acid and the alkali metal salts of these acids are normally used as inhibitors of unusual color-development but when these chelating agents are used in the present invention the resulting heat-sensitive recording sheets cannot simultaneously satisfy the three desired product requisites, that is, stability of the coating agent, shelf life of the heat-sensitive recording sheet and the desired characteristics of the recorded images (sharpness, contrast and color-forming sensitivity). On the contrary, the heat-sensitive recording sheets according to the present invention in which ethylenediamine tetraacetic acid or the alkali metal salts thereof are employed as the inhibitor can simultaneously satisfy the above-mentioned three desired requisites.

The proportions of components A, B and C are not critical, but it is preferred to use 100 parts by weight of component A, 10 - 500 parts by weight of component B and 1 - 50 parts by weight of component C.

The color tone of the print image obtained by using the heat-sensitive recording sheet of this invention is dark black and the print image is sharp and clear. Therefore, the recording sheet, having print images according to this invention, can be used as an original for reproduction or printing by diazograph, electrostatography and electrophotography.

According to another aspect of this invention, white pigments such as zinc white, white lead, titanium oxide, lithopone, alumina white, calcium carbonate, white carbon, antimony white, basic lead sulfate, lead silicate, zirconium oxide, tin oxide, barium sulfate, barium carbonate, and the like, can be added to the coating agent in order to convert the light brown color of the recording sheet resulting from the iron salt of the aliphatic acid to a whitish color without lowering the overall quality of the print image.

In the preparation of the heat-sensitive recording sheets of this invention, a binder solution is preferably utilized in addition to the color-forming components A and B, and the unusual color-forming inhibitor, i.e. component C. As the binder component, any well-known binder can be utilized. These include, for example, gelatin, polyvinyl alcohol, polyvinyl butyral, polyacrylic acid ester, polyacrylamide, polyvinylacetate, polyvinyl chloride, polystyrol, methylcellulose, ethylcellulose, polyamide resin, petroleum resin, terpene resin and silicon resin. As a solvent, any well-known solvent can be utilized such as water, alcohols such as methyl alcohol, ethyl alcohol, and isopropyl alcohol, ketones such as acetone and methylethyl ketone, esters such as ethyl acetate, aliphatic hydrocarbons such as hexane, heptane and petroleum benzine, halogen compounds such as methylene chloride and benzylchloride

and aromatic hydrocarbons such as benzene, toluene and xylene.

It is also preferable to add a solid fatty acid and/or wax to the formulations for the purpose of controlling the color-forming sensitivity and the sharpness. Examples of suitable solid fatty acids include stearic acid and palmitic acid. Examples of suitable waxes include carnauba wax, sperm aceti, paraffin wax, ceresine wax, microcrystalline wax, fatty acid amide wax, hardened castor oil, and specific synthetic wax.

The heat-sensitive recording sheets of this invention may be prepared by mixing a binder solution, a component A and a component C, grinding and dispersing the mixture by a ball-mill to form one suspension liquid, 15 and mixing a binder solution, a component B and a component C, grinding and dispersing the mixture by a ball-mill to form the other suspension, and then mixing the two suspension liquids with stirring to form a single coating liquid and finally coating the resulting 20 single coating liquid on a base sheet such as paper followed by drying the resulting coating.

The following examples will serve to illustrate but not to limit the invention. In the following examples, all parts are by weight.

25

#### EXAMPLE I

##### Formula for suspension liquid A:

|                 |          |
|-----------------|----------|
| Ferric stearate | 2 parts  |
| Stearic acid    | 10 parts |
| Vinylbutyral    | 10 parts |
| Methyl alcohol  | 20 parts |
| Ethyl acetate   | 50 parts |

##### Formula for suspension liquid B:

|                    |          |
|--------------------|----------|
| 8-hydroxyquinoline | 2 parts  |
| Ethylenediamine    |          |
| tetraacetic acid   | 2 parts  |
| Vinylbutyral       | 10 parts |
| Methyl alcohol     | 20 parts |
| Ethyl acetate      | 50 parts |

Each of the above-mentioned compositions were prepared in a ball-mill and the resulting suspension liquids

40 A and B were mixed by an agitator to form a homogeneous liquid coating agent. This coating agent was applied to a white paper to form a coating of 5  $\mu$  in thickness and dried at a temperature below 40°C. The resulting recording sheet gave a clear black image upon heating at a temperature higher than 80°C for 0.05 second.

The coating agent is stable and can be stored for a period of over one week and the heat-sensitive recording sheet itself is also stable and possesses a long shelf life.

50

#### EXAMPLE II

##### Formula for suspension liquid A:

|                    |          |
|--------------------|----------|
| Ferrous palmitate  | 3 parts  |
| Behenic acid       | 8 parts  |
| Ethylcellulose     | 8 parts  |
| Methylethyl ketone | 60 parts |

##### Formula for suspension liquid B:

|                                    |          |
|------------------------------------|----------|
| 5-chloro-7-iodo-8-hydroxyquinoline | 3 parts  |
| Disodium ethylenediamine           | 4 parts  |
| tetraacetate                       |          |
| Ethylcellulose                     | 10 parts |
| Methylethyl ketone                 | 60 parts |

60 The above-mentioned compositions were treated in the same manner as in Example I to form suspension liquids A and B and were applied to a white paper to produce a recording sheet. The resulting recording sheet gave a clear black image upon heating at a temperature

over 100°C for 0.05 second. Stability of the coating agent and stability of the heat-sensitive recording sheet are as good as those in Example I.

We claim:

1. A heat-sensitive recording sheet containing a coating layer consisting essentially of a uniform dispersion of particles of

- a. at least one iron salt of an aliphatic acid;
- b. at least one halogenated 8-hydroxyquinoline; and
- c. an inhibitor of unusual color-development selected from the group consisting of ethylene diamine tetraacetic acid and alkali metal salts thereof.

2. The heat-sensitive recording sheet of claim 1 wherein the aliphatic acid is an aliphatic carboxylic acid containing from about 8 to 24 carbon atoms.

3. The heat-sensitive recording sheet of claim 1 wherein the iron salt of the aliphatic acid is ferric stearate.

4. The heat-sensitive recording sheet of claim 1 wherein the iron salt of the aliphatic acid is ferrous palmitate.

5. The heat-sensitive recording sheet of claim 1 wherein the inhibitor of unusual color-development is ethylenediamine tetraacetic acid.

6. The heat-sensitive recording sheet of claim 1

15

10

15

20

25

wherein the inhibitor of unusual color-development is disodium ethylenediamine tetraacetate.

7. The heat-sensitive recording sheet of claim 1 wherein the coating layer contains a white pigment component.

8. The heat-sensitive recording sheet of claim 1 wherein the coating layer is deposited on a support.

9. The heat-sensitive recording sheet of claim 1 wherein the halogenated 8-hydroxyquinoline has the formula:



in which  $X_1$  is a halogen and  $X_2$  is a halogen or hydrogen.

10. The heat-sensitive recording sheet of claim 9 wherein  $X_1$  and  $X_2$  are similar or dissimilar and are selected from the group consisting of chlorine, bromine and iodine.

\* \* \* \* \*

30

35

40

45

50

55

60

65